

## UNITED STATES PATENT OFFICE

2,085,675

SAFETY PAPER AND METHOD OF MAKING  
SAMEFrancis L. Simons, Needham, Mass., assignor to  
George La Monte & Son, Nutley, N. J., a corpora-  
tion of New JerseyNo Drawing. Application February 4, 1935  
Serial No. 4,872

8 Claims. (Cl. 91—67.95)

This invention relates to safety paper including fraud preventing writing material made of paper or other substance or composition adapted for the printing or lithographing or for the inscription of writing or other mark or legend thereon and for use for example in the manufacture of checks, drafts, bonds, stock certificates or other instruments which it is desired to have protected against fraudulent alteration and methods of making such safety paper. This invention relates primarily to safety paper having incorporated therein by impregnation or superficial application either continuously or locally a chemical compound which is adapted upon application of a chemical ink eradicator thereto, to result in a disfiguring stain of a relatively permanent and indelible character which renders apparent attempts that are made to alter the safety paper by the use of a chemical ink eradicator.

It is the purpose of this invention to afford chemicals which when incorporated in safety paper develop disfiguring stains of a particularly vivid and permanent character upon the application of a chemical ink eradicator thereto. It is a further purpose of this invention to afford a chemical which when incorporated in safety paper does not discolor undesirably on aging due to premature development of color as the result of such causes as exposure to air and/or to light.

I have found that protection of a very desirable type can be afforded in safety paper by incorporating therein a mono-nitrogen substituted naphthylamine. Such compounds when incorporated in safety paper and treated with a bleach type of ink eradicator such as the ink eradicators extensively used at the present time containing hypochlorite solution or bleaching powder adapted to give up free chlorine, have been found to develop colors which are very vivid and give a very pronounced indication that attempt has been made to alter the safety paper. The colors so developed are likewise of a relatively permanent character as they are resistant to acids and alkalis and to reducing agents. Likewise such chemical compounds have been found to be highly stable on aging, that is, they do not tend to change color upon standing and/or exposure to light. Moreover, many of such substances are substantially colorless, that is, they do not tend to impart noticeable color to safety paper in which they are incorporated in proportions desirable for developing warning color indicia in the safety paper upon the application

of a chemical ink eradicator thereto. In this connection it may be stated that development of color includes change from a colorless substance to a colored substance, intensification of color or change from one color to another color. In the usual case the materials mentioned above change from a substantially colorless state or very slightly colored state to a very pronounced color. Normally it is regarded as preferable to employ substantially colorless compounds adapted to exhibit a decided color development when treated with a chemical ink eradicator.

By mono-nitrogen substituted naphthylamine it is meant that one only of the hydrogen atoms in the amino group has been replaced by an aliphatic, heterocyclic or aromatic substituent.

The formulae for naphthylamine may be written in either of the following ways, namely,



or



A more condensed formula covering both the alpha and beta naphthylamines may be written as follows:



wherein one R radical is the radical NH<sub>2</sub> and the remaining R radicals are hydrogen. The alpha ( $\alpha$ ) and beta ( $\beta$ ) positions have been indicated in the general formula and it is apparent that the NH<sub>2</sub> group can occupy either an  $\alpha$  or  $\beta$  position.

In mono-nitrogen substituted naphthylamines the —NH<sub>2</sub> group becomes the group



X being any aliphatic, aromatic, or heterocyclic

5

10

15

20

25

30

35

45

50

55

substituent for one of the hydrogen atoms of  $-\text{NH}_2$  group. Such aliphatic, heterocyclic and aromatic substituents include aliphatic, heterocyclic and aromatic hydrocarbon radicals, acidic derivatives of such hydrocarbon radicals, salts of said acidic derivatives, basic derivatives of such hydrocarbon radicals, and salts of said basic derivatives. By acidic derivative it is understood that a hydrogen atom of the hydrocarbon radical 5 is replaced by an acidic radical such as  $\text{SO}_3\text{H}$  (sulphonic);  $\text{NO}_2$  (nitro);  $\text{COOH}$  (carboxyl), or  $\text{Cl}$ ,  $\text{Br}$  or  $\text{I}$  (halogen). For the purposes herein set forth the  $\text{OH}$  (hydroxyl) radical may be included in the acidic group. The salts of such 10 acidic derivatives are the salts of alkali metals e. g. sodium and potassium and other salt forming alkaline earth and heavy metals. The term salt also includes organic salts or esters such as methyl, ethyl, phenyl, etc. By basic derivative it 15 is understood that a hydrogen atom of the hydrocarbon radical is replaced by a basic radical such as  $\text{NH}_2$  (amino). These basic derivatives form ammonium type salts such as the sulphates, hydrochlorides, acetates, oxalates, and the like.

20 25 In mono-nitrogen substituted naphthylamines which may be used according to this invention, the R radicals other than the



radical may be not only hydrogen but also an aliphatic, aromatic or heterocyclic substituent as above defined. Moreover, the mono-nitrogen 35 substituted naphthylamines which may be used in the practice of this invention may include more than one



group.

Likewise any one or more of the R radicals other than the



radical in mono-nitrogen substituted naphthylamines may be an acidic radical or a salt thereof or a basic radical or a salt thereof as above described only in such case the radical or radicals are attached directly to one or more carbon atoms of the naphthyl nucleus instead of to a carbon atom of a hydrocarbon substituent.

50 55 Mono-nitrogen substituted naphthylamines as referred to herein, include salts thereof such as the sulphates, hydrochlorides, oxalates, acetates and the like which salts may likewise be employed in the practice of this invention.

60 Certain mono-nitrogen-substituted naphthylamines which are preferably employed in the practice of this invention may be indicated by the formula



70 wherein one R radical is



X being any aliphatic, aromatic, or heterocyclic substituent. Preferably X is a hydrocarbon radical and of the hydrocarbon radicals aromatic and heterocyclic radicals are further to be preferred. It is likewise preferable that the remaining R radicals be any radical selected from the group consisting of



10

as above defined, hydrogen, hydrocarbon radicals, acidic derivatives of hydrocarbon radicals, salts of said acidic derivatives, basic derivatives of said hydrocarbon radicals, salts of said basic derivatives, acidic radicals, salts of said acidic radicals, basic radicals, and salts of said basic radicals. As above mentioned, the mono-nitrogen substituted naphthylamines which may be employed in the practice of this invention also includes salts formed with the basic



15

group.

In the foregoing description the hydrocarbon radicals may be radicals such as methyl, ethyl, propyl, etc., as well as aromatic radicals such as phenyl, naphthyl, tolyl, etc. and heterocyclic radicals are pyridyl, pyrrol, quinolyl, etc. It is not regarded as necessary to list the names of substituted naphthylamines having such radicals. In the case of the phenyl radical, for example, as contained in mono-nitrogen substituted naphthylamine the name of the compound is N-phenyl-alpha-naphthylamine or N-phenyl-beta-naphthylamine, the N symbol indicating that the phenyl is attached to the N atom of the naphthylamine. The same applies in applying nomenclature to substituted naphthylamines containing other radicals above mentioned.

Referring to acidic substituents and acidic derivatives of hydrocarbon substituents the sulphonic and carboxyl derivatives are preferred. Also the alkali metal salts e. g. sodium or potassium of acidic derivatives are preferred where water solubility is desired.

The preparation of safety paper embodying this invention can be practiced in several ways. The 50 naphthylamines above mentioned which are insoluble in water may be incorporated in safety paper by mixing the same with the paper fibre during the beating operation which forms a step in the paper making process. The chemical may 55 be added in the form of a dry powder, for example, as the chemicals above mentioned are very stable and will not be altered during the beating operation or during the subsequent steps of the paper making process. The chemical compound in such case is carried down into the finished paper so that when attempt is made to alter a legend on the paper by using a chemical ink eradicator such as a bleach, the paper will 60 develop a pronounced color which affords a warning indicia. In the case of the N-phenyl-naphthylamines, and other naphthylamines of an analogous character about 2% to 10% of the chemical on the dry weight of the paper may be used. Of course, greater or lesser amounts can be 65 used, depending on the amount of color developed by the application of a chemical ink eradicator to the substance selected and the intensity of color that is desired in the warning stain. Normally, the greater the amount of safety chem- 70

65

75

ical in safety paper, the more intense will be the color that is developed when a chemical bleaching material is applied to the safety paper.

Alternately, the safety chemical may be dissolved in a suitable solvent therefor. Thus many of the mono-nitrogen substituted naphthylamines above mentioned are soluble in solvents, such as acetone, ethyl alcohol, benzene and the like or mixtures thereof. A solution of the safety chemical may be applied in any suitable manner as by dipping, spraying, etc. The concentration of the solution is preferably such that about 2% to 10% of the chemical on the weight of the paper will be retained after the solvent has been evaporated from the paper. When a water soluble naphthylamine derivative is used water may be used as a solvent.

The safety chemicals by the methods above described or by any other method of impregnation or surface application, can be impregnated in the body of the safety paper or may be applied to the surface thereof and while it is preferable to have all parts of the safety paper react similarly to chemical ink eradicators due to the uniform distribution of the safety chemical therein, the safety chemical can be applied locally as by printing or other suitable method. In any event, safety paper carrying a safety chemical herein described is to be regarded as having any such safety chemical incorporated therein. It will be understood that this invention is applicable among other fields of application in connection with plain white paper as well as tinted paper

or paper having surface markings thereon. It is likewise applicable when a tint in the paper is delible under the action of chemical ink eradicators and/or when the surface marking or tinting is removable by mechanical erasure.

While this invention has been described in connection with certain specific examples thereof, it is to be understood that this has been done merely for the purpose of illustration and that the scope of this invention is to be governed by the following claims.

I claim:

1. A safety paper having incorporated therein a mono-nitrogen substituted naphthylamine.
2. A safety paper having incorporated therein N-phenyl-naphthylamine.
3. A safety paper having incorporated therein N phenyl naphthylamine sulphonic acid.
4. A safety paper having incorporated therein N phenyl amino naphthylamine.
5. A method of making safety paper which comprises incorporating in paper N-phenyl naphthylamine.
6. A method of making safety paper which comprises incorporating in paper N-phenyl naphthylamine sulphonic acid.
7. A method of making safety paper which comprises incorporating in paper N-phenyl amino naphthylamine.
8. A method of making safety paper which comprises incorporating in paper a mono-nitrogen substituted naphthylamine.

FRANCIS L. SIMONS.

#### Certificate of Correction

Patent No. 2,085,675.

June 29, 1937.

FRANCIS L. SIMONS

It is hereby certified that error appears in the printed specification of the above numbered patent requiring correction as follows: Page 2, first column, line 45, for the formula



read:



and that the said Letters Patent should be read with this correction therein that the same may conform to the record of the case in the Patent Office.

Signed and sealed this 1st day of March, A. D. 1938.

[SEAL]

HENRY VAN ARSDALE,  
Acting Commissioner of Patents.

ical in safety paper, the more intense will be the color that is developed when a chemical bleaching material is applied to the safety paper.

Alternately, the safety chemical may be dissolved in a suitable solvent therefor. Thus many of the mono-nitrogen substituted naphthylamines above mentioned are soluble in solvents, such as acetone, ethyl alcohol, benzene and the like or mixtures thereof. A solution of the safety chemical may be applied in any suitable manner as by dipping, spraying, etc. The concentration of the solution is preferably such that about 2% to 10% of the chemical on the weight of the paper will be retained after the solvent has been evaporated from the paper. When a water soluble naphthylamine derivative is used water may be used as a solvent.

The safety chemicals by the methods above described or by any other method of impregnation or surface application, can be impregnated in the body of the safety paper or may be applied to the surface thereof and while it is preferable to have all parts of the safety paper react similarly to chemical ink eradicators due to the uniform distribution of the safety chemical therein, the safety chemical can be applied locally as by printing or other suitable method. In any event, safety paper carrying a safety chemical herein described is to be regarded as having any such safety chemical incorporated therein. It will be understood that this invention is applicable among other fields of application in connection with plain white paper as well as tinted paper

or paper having surface markings thereon. It is likewise applicable when a tint in the paper is delible under the action of chemical ink eradicators and/or when the surface marking or tinting is removable by mechanical erasure.

While this invention has been described in connection with certain specific examples thereof, it is to be understood that this has been done merely for the purpose of illustration and that the scope of this invention is to be governed by the following claims.

I claim:

1. A safety paper having incorporated therein a mono-nitrogen substituted naphthylamine.
2. A safety paper having incorporated therein N-phenyl-naphthylamine.
3. A safety paper having incorporated therein N phenyl naphthylamine sulphonic acid.
4. A safety paper having incorporated therein N phenyl amino naphthylamine.
5. A method of making safety paper which comprises incorporating in paper N-phenyl naphthylamine.
6. A method of making safety paper which comprises incorporating in paper N-phenyl naphthylamine sulphonic acid.
7. A method of making safety paper which comprises incorporating in paper N-phenyl amino naphthylamine.
8. A method of making safety paper which comprises incorporating in paper a mono-nitrogen substituted naphthylamine.

FRANCIS L. SIMONS.

#### Certificate of Correction

Patent No. 2,085,675.

June 29, 1937.

FRANCIS L. SIMONS

It is hereby certified that error appears in the printed specification of the above numbered patent requiring correction as follows: Page 2, first column, line 45, for the formula



read:



and that the said Letters Patent should be read with this correction therein that the same may conform to the record of the case in the Patent Office.

Signed and sealed this 1st day of March, A. D. 1938.

[SEAL]

HENRY VAN ARSDALE,  
Acting Commissioner of Patents.

**Certificate of Correction**

Patent No. 2,085,675.

June 29, 1937.

**FRANCIS L. SIMONS**

It is hereby certified that error appears in the printed specification of the above numbered patent requiring correction as follows: Page 2, first column, line 45, for the formula



read:



and that the said Letters Patent should be read with this correction therein that the same may conform to the record of the case in the Patent Office.

Signed and sealed this 1st day of March, A. D. 1938.

[SEAL]

**HENRY VAN ARSDALE,**  
*Acting Commissioner of Patents.*